

Feb. 1, 1938.

F. TAVIN ET AL

2,106,819

METHOD FOR MAKING TRANSPARENT PUFFING

Filed July 26, 1937

FIG. 1



2

FIG. 2



FIG. 3



FIG. 5



FIG. 4



BY

INVENTORS  
FRANK TAVIN & HANS HAAS

*Irving Seidman*  
THEIR ATTORNEY.

## UNITED STATES PATENT OFFICE

2,106,819

METHOD FOR MAKING TRANSPARENT  
PUFFING

Frank Tavin, New York, N. Y., and Hans Haas, Freehold, N. J., assignors to Isidore Eckstein and Morris Landau, doing business as I. D. Manufacturing Co., New York, N. Y.

Application July 26, 1937, Serial No. 155,654

5 Claims. (Cl. 2—278)

This invention relates to a method of making translucent or transparent puffing in materials.

Broadly, it is an object of this invention to provide a new method of decorating material for 5 ladies' wearing apparel, millinery, bed quilts, draperies, table covers, and other like articles.

More specifically, it is an object of this invention to provide a method of making a translucent and transparent puffing for material in order to 10 decorate such fabrics, thus increasing the saleability of such materials.

Another object is to provide for a simple and economical method of decorating ladies' dresses, gowns and wraps, whereby a design can be made 15 to fit each portion of the garment, such as the front, back, sleeves and borders, so that the design will harmonize with the style and character of the garment.

Another object is to provide a transparent or 20 translucent puffing in various designs in materials, whereby a colored thread or threads are introduced between two or more layers of material, so that the colored thread or threads are visible through the material to produce interesting and 25 artistic colored ornamentation and designs.

Another object is to create transparent or translucent puffing ornamentation so that ladies' jackets can be made reversible, each side presenting a different color scheme.

30 Another object is to provide for double faced designs for translucent or transparent embroidered materials.

Another object is to provide for translucent or 35 transparent puffing to ornament and decorate pile velvets. Another object is to provide pocket sections to receive colored materials, whereby each pocket section receives an individual colored thread that acts as a puffing to create a puffed, colored, ornamental fabric.

40 These and other advantages, capabilities and features of the invention will appear from the subjoined detailed description with the aid of the accompanying drawing and more particularly pointed out in the claims appended hereto, in 45 which:

Fig. 1 illustrates a plan view of a piece of material showing a design of transparent puffing.

Fig. 2 is a section taken through line 2—2 of Fig. 1.

50 Fig. 3 shows a section of three layers of material joined together with stitching having double pocket sections for puffing.

Fig. 4 illustrates a plan view of a piece of material showing a design of transparent puffing 55 upon a pile velvet material.

Fig. 5 is a section taken through line 5—5 of Fig. 4.

Referring to the drawing, numeral 10 represents a thin, translucent or transparent material such as mouseline de soie or silk comprising the 5 face of the article to be decorated. The backing material 11, which may be of the same character as the face material 10, is sewn to face material 10 by stitching along lines representing a pleasing design, such stitching being indicated at 12, 13, 10 14, 15 and 16. Any desired type of design can be traced upon material 10 so that any portion of a garment may have a design to fit such portion, such as the front and collar or the sleeves. The stitching together of materials 10 and 11 creates 15 pocket sections 17 between the stitching lines as shown in Fig. 2.

In order to insert colored thread 18 into pockets 17, a hollow needle is used having an opening through its longitudinal center through which is 20 fed the colored thread 18 used for puffing. One end of the hollow needle is inserted through the material 11 and the opposite end is connected to a rubber tube leading to an air tank containing air under pressure. When the operator steps upon 25 a foot pedal, a blast of air is released and forces the colored thread 18 through the hollow shaft of the needle and into the pocket 18, thus filling the entire pocket section with colored thread.

Each section may contain a differently colored 30 thread in any desired combination of colors or a twisted thread of two or more colors in order to obtain a multicolored effect in each pocket section. The colored thread in the different pockets 35 17 is readily seen through the transparent or translucent materials 10 and 11, thus producing a puffed design on the material of interesting and pleasing color combination.

In Fig. 3, material 19 is inserted between materials 10 and 11 and all three materials are sewn 40 together by stitching 12, thus creating double pocket sections 20 and 21. A colored thread is then blown into pocket section 20 in the same manner as explained above and a differently colored thread is blown into pocket section 21. 45 Thus, the colored design appearing through the material 10 can be different than the colored design appearing through material 11. Material 19 may be opaque so that the colored threads used for puffing will not show through the opposite 50 side. Thus, reversible jackets can be made with different color schemes on each side. If desired, material 19 may also be translucent or transparent so that the colored thread in pocket 20, for example, may influence and blend with colored 55

thread in pocket 21. Thus, if pocket 20 contains a yellow thread for puffing, and pocket 21 a blue thread, the combination of color of both threads will produce a green effect.

5 Fig. 4 pictures a flower design upon a pile velvet material 22. Every pile velvet contains a back and the strands comprising the pile stand at right angles to the back. It is necessary to remove the pile strands of the velvet in desired portions of 10 the velvet material so that the back only will remain. In order to produce the flower shown in Fig. 4 and bounded by stitching 23, it is necessary to remove all the pile within the area. In 15 the method to be described, a velvet is used consisting of a back of natural silk and pile strands of wood silk and the mixture is applied to the back of the velvet.

This mixture is made by boiling gum tragacanth and adding about 11% of aluminum chloride and 20  $\frac{1}{4}$  of 1% of glycerine.

The mixture is heated between 150° and 190° 25 Fahrenheit and stirred during the heating process, preferably with a mechanical mixer, until it has the consistency of molasses. Distilled water is added to thin the mixture. The mixture is then cooled and placed in jars ready for use. When the cool mixture is actually applied to the 30 back of the velvet, about 2% aluminum chloride is added to the mixture for easier application.

35 The velvet is placed face down upon a table and a design is outlined upon the back of the velvet. The aforementioned mixture is then applied only upon the back of the velvet and wherever it is desired to remove the pile of the velvet. For quantity work a silk screen containing the 40 design may be used and the mixture moved over this silk screen with a squeegee so that the mixture comes through the silk screen and produces the design upon the back of the velvet.

45 The mixture is allowed to dry thoroughly and harden. To speed production, the velvet containing the mixture may be baked in an oven. The velvet is then pinned face up upon a cloth covered table and a small vacuum cleaner containing a brush is passed over the surface of the velvet. The nap of the velvet where the mixture was applied will thus be removed and the mixture which has become crystallized will also be removed. The back of the velvet consisting of 50 natural silk will remain.

A thin backing material 28 shown in Fig. 4 is 55 sewn to the back of the velvet 22 by stitching along lines representing the flower design or any other design, such stitching being indicated at 23, 24, 25 and 26. The stitching together of backing material 28 to the back of the velvet 22 creates pocket sections 29 between stitching lines as shown on Fig. 5.

60 Colored threads are then blown into pockets 29 through a hollow needle as above described, creating colored puffing which is readily visible through the back of the velvet from which the pile had been removed. The ornamented material is then used for various kinds of ladies' 65 wearing apparel and other articles.

While in the foregoing the preferred embodiments of the invention have been described and shown, it is understood that the construction is susceptible to such alterations and modifications as fall within the scope of the appended claims. 5

We claim:

1. A method of producing translucent puffing consisting of joining together two pieces of material by stitching, said stitching creating pockets to receive different colored threads by inserting 10 a hollow needle through the material into said pockets and forcing a blast of air through said hollow needle whereby a colored thread within said hollow needle is forced into said pockets to produce a translucent, ornamental, colored, puffed 15 fabric.

2. A method of producing puffed material consisting of joining together a translucent facing material and a backing material by stitching to create pocket sections, inserting a hollow needle 20 through the backing material and blowing a colored thread through the needle and into said pocket sections to produce a puffed material of colored design.

3. A method of producing puffed goods upon 25 velvets of wood silk pile and natural silk back consisting of tracing the design upon the back of the velvet, applying a mixture of gum tragacanth, 11% of aluminum chloride and  $\frac{1}{4}$  of 1% of glycerine upon said design, allowing said mixture to dry, placing said velvet pile face up upon a table, removing the treated wood pile from said velvet leaving the natural silk back exposed, applying a backing material to the back of said 30 velvet over the pile removed portions by stitching, 35 stitching through said exposed pile velvet back and said backing material to create pocket sections, inserting a hollow needle through the said backing material and blowing a thread through the needle and into said pocket sections to produce a puffed material of design determined by 40 said stitching upon said pile velvet material.

4. A method of producing puffing consisting of joining together two pieces of material by stitching, said stitching creating pockets to receive 45 filling material by inserting a hollow needle through the material into said pockets and forcing a blast of air through said hollow needle, whereby a filling material within said hollow needle is forced into said pockets to produce a 50 puffed fabric.

5. A method of producing puffed goods upon 55 velvets and wood silk pile and natural silk back, consisting of tracing the design upon said velvet, treating the fabric within said design with a dissolving mixture to remove the treated wood pile from said velvet, allowing the natural silk back to remain exposed, stitching a backing material to the back of said velvet to conform to said design forming a plurality of pockets, thereafter blowing a thread into said pockets through a hollow needle inserted therein to produce a 60 puffed material.

FRANK TAVIN.  
HANS HAAS.

65